

Dec. 24, 1963

H. T. RANDALL

3,115,438

## METHOD OF COATING PAPER

Filed Aug. 11, 1960



INVENTOR.  
HERBERT T. RANDALL

BY Donald A. Hoes  
ATTORNEY

1

3,115,438

## METHOD OF COATING PAPER

Herbert T. Randall, Hamilton, Ohio, assignor to Champion Papers Inc., Hamilton, Ohio, a corporation of Ohio

Filed Aug. 11, 1960, Ser. No. 49,088  
5 Claims. (Cl. 162—184)

This invention relates to the manufacture of "cast" surface coated paper.

In the prior art methods of producing cast coated paper it has been the practice to apply a wet coating material to a previously and separately formed paper sheet followed by drying the coating in intimate contact with a solid casting surface such as a chromium plated drum. Such a process is disclosed in the U.S. patent to Bradner, No. 1,719,166. Although this process has been successfully practiced commercially for a number of years, it nevertheless suffers from several disadvantages. One difficulty is the fact that in order to obtain a high gloss smooth sheet it is necessary to apply an excessively heavy weight of coating either in the casting step itself or in combination with conventional coating operations prior to the casting step. This is because of the fact that in the manufacture of the raw stock, defects are often produced such as cockle, fuzz, poor formation and "grainy edges," which are difficult to cover. Calendering of such a raw stock to reduce these deficiencies may result in crushed streaks or blotchy areas. Furthermore, the application of a heavy layer of coating to cover these defects requires a lessening of the casting speed and often results in a weak and brittle sheet having poor fold properties.

A second disadvantage of the casting procedure as heretofore employed is the fact that to a large extent it requires an undue number of steps and an extensive amount of equipment. Thus it has heretofore been the practice to prepare the paper web such as on a Fourdrinier or cylinder machine followed by drying it and winding it up into suitable rolls. When the paper is then cast coated it is desirable to rewet the paper such as on the casting drum in order to avoid a problem of curling. The latter is disclosed in U.S. patent to Warner, No. 2,360,919. The initial drying on the paper machine is therefore an extra operation which, for economical reasons, should desirably be avoided.

A further difficulty which has been encountered in the prior art process of cast coating of paper is the fact that it is difficult to closely control the uniformity of the coating which is applied to the stock. This is for the reason that the stock, being substantially dry, is not uniformly absorbent to the coating.

An object of this invention therefore is an improved method of cast coating by utilizing undried cellulosic web stocks.

In accordance with this invention it has been found that the above noted disadvantages are overcome by cast coating a wet paper web containing a critical amount of moisture as it comes from the paper forming machine. According to this method a freshly formed paper web is led from the paper machine through an initial moisture reducing section and then placed in contact with an aqueous coating composition containing adhesive and a finely divided pigment material, followed by drying the web against a smooth casting surface.

The FIGURE illustrates apparatus suitable for carrying out the process of this invention.

A web of paper 10 is formed in any conventional paper forming machine 11. For simplicity the latter is exemplified as a cylinder machine in the drawing. It is to be understood that a Fourdrinier may be used equally as

2

well. A particularly suitable apparatus, owing to its relatively small size and wide versatility, is the Rotoformer unit manufactured by the Sandy Hill Iron and Brass Works of Hudson Falls, New York, and described in

5 Paper Mill News, vol. 82, No. 28, pages 14 and 18. The Rotoformer is particularly advantageous for use in this invention since its vacuum sections facilitate control of the moisture content of the web. A roll 12 aids in removing the paper web from the paper forming machine.

10 A suction press is illustrated by rolls 13 and 14. This may suitably be equipped with a vacuum pump to further reduce the water content of the web. A smooth press, as represented by rolls 15 and 16, may be provided in order to smooth the web by pressure. The roll 26 is a guide roll. The drums 27 are heated drying drums which also may be employed to reduce the moisture content of the web to the desired level. It is to be understood that any suitable means may be provided in order to control the moisture content. Thus, either the suction press or

15 the drying drums in the drawing may be dispensed with, used interchangeably or replaced by other suitable means provided that the moisture content of the web is properly controlled. Rolls such as 28 may be provided in order to guide the web to the coater 19. Preferably a moisture

20 measuring device is located ahead of the coater to automatically record the moisture content of the web. The coating applicator 19 may be any conventional coater such as a roll coater, an air knife coater, a doctor roll, etc. Roll 20 merely serves to press the coated web in contact with

25 the heated casting drum 21. The latter should have a smooth surface and for this reason a polished chromium surface is preferred. Nickel, brass and hard rubber are surfaces which also may be employed. Roll 22 permits

30 removal of the dried coated web from the casting drum and from there it is led to the windup reel 24 equipped with guide rolls 23 and 25. In view of the high water content of the web stock a felt (not shown in the drawing) will ordinarily be employed to support the web throughout all or a portion of its length as it passes from the paper

35 forming machine 11 until it reaches the casting drum 21. Various other supporting carriers, such as a rubber belt, may similarly be used for this purpose.

The coatings employed for producing the cast surface will ordinarily be aqueous dispersions of a finely divided 45 pigment together with an adhesive such as casein, soy protein, starch or a synthetic polymer emulsion. Examples of pigments include calcium carbonate, clay, titanium dioxide, etc. The solids content of the coating will usually be in the range of 25-65% by weight although it may contain more or less depending upon the desired thickness of the coating on the web. Usually it is desired to work within the range of 45-65% by weight solids content in order to give maximum coverage of the sheet.

55 Instead of coating the paper web and casting this against the drum it is also possible to coat the drum directly with the coating composition and to press the wet but uncoated web in contact with the coated drum. In this way it is possible to decrease substantially the amount of coating which is necessary to produce a high gloss cast finish. It is important that the coating on the drum is not dried to any appreciable extent, i.e., less than 20% water, before being contacted with the paper web or some of the advantages of the more uniform absorption 60 of coating into the web will not be realized.

Still another method of regulating the amount of coating which may be applied to the web involves precoating the freshly formed web prior to application of the coating for the casting operation. Thus, referring to 65 the drawing, it is for certain purposes desirable to position a precoater between guide rolls 23 and coating ap-

plicator 19 or between the paper machine 11 and the driers 27. Such a precoater can be the same or different from the coating applicator. The use of this additional coater makes possible the obtaining of sheets with a much higher total weight of coating than is possible by the single coating operation. The precoater should preferably employ the same coating which is to be later applied by the cast coater although different coatings of pigment and adhesive may also be used.

The moisture content of the web prior to cast coating must be continuously controlled in order to produce a satisfactory cast coated sheet. It is necessary that the moisture content of the web, between the time of formation and casting on the drum, be maintained at a sufficiently high level. A moisture content of at least about 20% by weight is generally desired for the freshly formed web. It will not usually be desirable to employ a web containing more than about 65% by weight of water. When the moisture content is greater than 65% adequate drying cannot be achieved at reasonable speeds on the casting drum. Moreover, with so much water the web is easily torn and makes handling difficult. Also, and most important, the quality of the coated sheet drops off sharply when the water content is more than 65% because of the voids created by the loss of water. When the moisture content of the sheet is below 20%, the fibers shrink, distort and stiffen and it becomes increasingly difficult to thoroughly wet the surface of the web with coating. Due to the lack of absorbency of this relatively low moisture content web, a uniform coating is not readily obtained.

The casting of an undried sheet in accordance with this invention avoids the undesirable characteristics of cockle and grainy edges normally encountered in the preparation of raw stock for a conventional casting operation. In addition the wet casting permits flattening of the sheet against the drum surface with a minimum amount of pressure and with a minimum coating weight.

It has been found that the time required to completely dry a web which contains 20-65% by weight of moisture prior to being coated with an aqueous pigmented coating is not substantially greater than that which is required to dry a relatively moisture free web which has been coated with the same aqueous coating. The reason for this apparently lies in the fact that the web is so uniformly wet throughout its thickness that the water molecules are easily vaporized. Thus with a 12 foot diameter chromium surface casting drum heated to a temperature of 150-212° F. or more it is possible to operate at speeds up to 300 feet per minute. When the moisture content of the web is regulated to within the particularly desirable range of 45-60% by weight it is possible to operate at speeds even in excess of 300 feet per minute.

In order to facilitate removal of the cast sheet from the casting drum it is desirable to produce a monomolecular film of an oleaginous release agent on the surface of the drum as disclosed in the U.S. Reissue Patent to Montgomery No. 23,637, reissued March 24, 1953. The film of release agent is desirably formed by buffing the drum with the oleaginous material and by replenishing this by incorporating a small amount of the agent directly in the aqueous pigmented coating. The coatings employed in the aforesaid Montgomery patent are also suitable for use in the present invention.

Depending upon the speed of the casting drum and its temperature, the resulting cast sheets, after release from the drum, may still contain appreciable amounts of moisture. Thus a cast sheet can be made to release from the drum when the coating is dry although the web itself may still contain a relatively high amount of moisture, i.e., the total moisture content of the coated web can be in excess of 10% by weight with the bulk of this being present in the web, at least immediately after casting. The higher amount of moisture in the web makes it

possible to control the curling tendency of the paper by subjecting it to a further drying treatment. In addition the higher moisture content of the paper is desirable in certain printing operations.

It has surprisingly been found that cast coating of a freshly formed web in accordance with this invention produces a quite different and superior effect from that obtained by cast coating a relatively dry web or even a web which has been dried and subsequently rewet. The reason for this apparently resides in the fact that a freshly formed web has a uniform moisture content throughout its thickness which renders it uniformly absorbent toward the coating. When a sheet is once dried of moisture and later rewet, the moisture content throughout the thickness of the sheet is not uniform unless a lengthly period of time is provided in which the moisture content can come to equilibrium. Even then the shrinkage and distortion of the dried fibers cannot be fully corrected. The greater absorbency of a freshly formed web makes possible a sizeable increase in the speed of the coating operation.

The present invention has the additional advantage of permitting the application of much heavier coatings than has heretofore been possible by the conventional casting techniques. There is no difficulty in getting 20 pounds of coating per ream at the same solids content onto a sheet that would have given only 10 pounds per ream if the sheet were dried. The method of this invention permits the application to a single side of the paper of up to 40 pounds of coating per ream and even more.

By making the casting step a part of the paper making operation it is possible to provide for continuous inspection and for immediate correction of defects. In addition, the losses normally encountered in unwinding and rewinding the rolls and in the handling of the rolls in the extra steps of the conventional process are avoided.

The following examples will serve to illustrate the practice of the instant invention.

#### Example I

A conventional stock formed from a furnish of sulfate pulp fibers and weighing approximately 32 pounds per ream dry (500 sheets 25 x 38 inches) was led from the wire section of a Fourdrinier through a press section and to heated drier cylinders. The following samples were obtained with different moisture contents by varying the number of drying drums over which the web was passed.

| 50 | Sample   | Number of driers | Percent by weight moisture in web |
|----|----------|------------------|-----------------------------------|
|    | (a)----- | 1                | 58.2                              |
| 55 | (b)----- | 5                | 23.9                              |

The webs were each supplied to a roll coater which applied 21.4 pounds (dry) to sample (a) and 24.2 pounds (dry) to sample (b) of a coating comprising a mixture of:

| 60 | Ingredient:                                                                                                                 | Parts by weight |
|----|-----------------------------------------------------------------------------------------------------------------------------|-----------------|
|    | Clay (dry)-----                                                                                                             | 100             |
|    | Casein-----                                                                                                                 | 11              |
| 65 | Latex of a polymer of 40% by weight butadiene and 60% by weight styrene having a total solids content of 50% by weight----- | 7               |
|    | Oleic acid-----                                                                                                             | 1               |
|    | Sufficient water to dilute the coating to 62% total solids.                                                                 |                 |

The web in each case was then pressed against a rotating chromium surfaced drum heated to 150° F. which had initially been buffed to establish a film of release agent on its surface. The coated webs were each easily stripped from the drum when dry to produce an extremely glossy cast surface.

*Example II*

The procedure of Example I is repeated using a coating of the same formulation. A heavy stock weighing an average of about 110 pounds per ream dry (500 sheets 25 x 38 inches) and containing approximately 45% by weight moisture was taken from the first drier following the Fourdrinier. The coater applied about 14-15 pounds (dry) to sample (a) and about 25 pounds (dry) to sample (b). With sample (a) the chromium drum was heated to 204° F. whereas with sample (b) it was heated to 200° F. Each coated web stripped readily from the drum to produce a high gloss cast sheet when the coating was dry. At this stage sample (a) contained about 1.7% by weight of water while sample (b) contained nearly 20% water. Sample (b) was led through a heated drier to further reduce the moisture content to 3%.

Although the preferred embodiments of this invention have been disclosed, it will be obvious that many variations and changes can be made without departing from its intended scope.

I claim:

1. The method of producing cast coated paper which comprises forming a web from a furnish of water and pulp, partially drying said web to reduce the moisture content to no less than 20% by weight and no more than 65% by weight, thereafter contacting the web with

an aqueous coating composition comprising adhesive and finely divided pigment material, drying said web with said aqueous coating composition against a smooth casting surface and removing the dried coated web from said casting surface.

- 5 2. The method of claim 1 wherein the paper web is coated with the aqueous coating composition and then is pressed into contact with the casting surface.
- 10 3. The method of claim 1 wherein the paper web is pressed against a casting surface which has been coated with the aqueous coating composition.
- 15 4. The method of claim 1 wherein the casting surface is a polished chromium surface.
5. The method of claim 1 wherein the coated web is removed from the casting surface before the moisture content of the coated web is reduced below 10%.

## References Cited in the file of this patent

## UNITED STATES PATENTS

|    |            |                  |       |                |
|----|------------|------------------|-------|----------------|
| 20 | Re. 23,637 | Montgomery       | ----- | Mar. 24, 1953  |
|    | 2,032,211  | Hornbostel       | ----- | Feb. 25, 1936  |
|    | 2,772,604  | Muggleton        | ----- | Dec. 4, 1956   |
|    | 2,919,205  | Hart             | ----- | Dec. 29, 1959  |
| 25 | 3,024,160  | Kapral           | ----- | Mar. 6, 1962   |
|    | 3,044,896  | Warner           | ----- | July 17, 1962  |
|    | 3,054,716  | Bergstein et al. | ----- | Sept. 18, 1962 |